

106/84

Feb. 18, 1930.

S. RUBEN

1,747,649

METHOD OF MAKING A RESISTANCE ELEMENT

Filed Jan. 5, 1929

FIG.1.



FIG.2.



Inventor  
SAMUEL RUBEN

By his Attorney *W.L. Cease*

XR

## UNITED STATES PATENT OFFICE

SAMUEL RUBEN, OF NEW YORK, N. Y., ASSIGNOR TO RUBEN PATENTS COMPANY, OF NEW YORK, N. Y., A CORPORATION OF DELAWARE

## METHOD OF MAKING A RESISTANCE ELEMENT

Application filed January 5, 1929. Serial No. 330,608. 201-68

This invention relates to a method of making a resistance element and more particularly it relates to a method of applying a resistance coating upon the surface of a conductive member of a resistance device employing surface pressure changes for current control.

The object of the invention is the provision of a resistance element for controlling current between a low minimum and a relatively high maximum value in accordance with pressure variations between the elements.

It is old in the art to employ a carbon disc as the resistance element between conductive plates in a variable pressure resistance device, 15 in the use of which various disadvantages exist, such as fragility and the relatively high resistance at maximum pressure, due to the necessary thickness of the disc material.

I have found that highly satisfactory results are obtained in variable pressure resistance devices in which relatively high temperatures develop, by employing as the resistance element a mixture of gas carbon and a suitable inorganic binder applied as a coating upon conductive plates, such as iron or aluminum, which is then dried and heated to effect partial volatilization of the binder, leaving a hard substance, and thereafter compressed. In this way is obtained the desired even distribution of a durable, adherent compressed coating which has a hard, smooth surface, insuring evenly distributed surface contact with a like coating upon another conductive plate or directly with such a plate, thereby preventing current localization. The thickness of the coating is determined by the energy to be applied. In a device employing a metal coating so produced the resistance value at maximum pressure is very low, due 40 to the metal base and the thin layer of the resistance material.

The preferred coating consists of a mixture of gas carbon, and an inorganic binder applied to a thoroughly cleansed iron surface.

45 After drying, the metal disc with its coating is subjected to a temperature of approximately 500° C. and then passed between rollers compressing the coating and reducing its thickness, and producing a smooth surface of 50 uniform thickness. A preferred mixture is

gas carbon with 30% silicate. Such a coating has been found to have greater negative pressure resistance than that of a graphite coating or of the carbon discs.

For a better understanding of the invention reference is made to the accompanying drawings which illustrate one embodiment of the invention. In Figs. 1 and 2, C represents the carbon coating mixture applied to opposite surfaces of the aluminum plate P. 6

What I claim is:

1. The method of making an element for a pressure controlled rheostat, which consists in applying to the surface of a conductive body a mixture containing gas carbon and an inorganic binder, drying the coating, heating it to approximately 500° C. and passing the coated body between compression rollers. 61

2. The method of making a resistance element for a pressure controlled rheostat, which 70 consists in applying to the surface of a metallic body a layer of gas carbon mixed with an inorganic binder, partially volatilizing the binder and compressing the coated element so as to produce a uniformly distributed layer 75 of the resistance metal.

3. The method of making a resistance element for a pressure controlled rheostat, which consists in coating the surface of a conductive body with a mixture containing 80 gas carbon and a silicate and heating the coating until a partial volatilization of the silicate occurs, and compressing the coating.

4. The method of making a resistance element for a pressure controlled rheostat which 85 consists in coating the surface of a conductive body with a mixture containing 70% gas carbon and 30% silicate heating the coating until a partial volatilization of the silicate occurs and compressing the coating. 90

In testimony whereof SAMUEL RUBEN has signed his name to this specification this 27th day of December, 1928.

SAMUEL RUBEN.

95

100